

May 12, 1959

OSAMU MADONO

2,886,428

METHOD OF MANUFACTURING DUCTILE HIGH ALUMINUM IRON ALLOY

Filed April 1, 1957



INVENTOR

BY O. Madono  
Wendroth, Lind & Ponack  
Atlys

# United States Patent Office

2,886,428

Patented May 12, 1959

1

2,886,428

## METHOD OF MANUFACTURING DUCTILE HIGH ALUMINUM IRON ALLOY

Osamu Madono, Kumagaya-City, Japan

Application April 1, 1957, Serial No. 649,667

Claims priority, application Japan December 26, 1956

5 Claims. (Cl. 75—12)

The present invention relates to a method of manufacturing ductile high aluminum-iron alloys by means of a consumable electrode type arc furnace, having an advantage of the freedom of selection of the starting materials, which permits carbon or alloy steel to be more effectively used than electrolytic or ingot iron. In spite of the freedom of the selection of the starting materials, the products, compared with the existing high aluminum-iron alloys made by other methods, are more ductile, and yet have high strength, heat resistance, oxidation resistance, together with excellent magnetic properties and high electrical resistance.

It has been well-known for many years that aluminum greatly improves the above various properties of ferrous alloys. But their use is limited because of the difficulty of producing the inherently brittle aluminum ferrous alloys in usable form. That is, ferrous alloys with an aluminum content less than about 5% may be either hot or cold worked without difficulty; ferrous alloys containing aluminum in an amount more than about 5% becomes too brittle for cold working. The ductility of the aluminum ferrous alloys is strongly influenced by the presence of extremely small amounts of carbon, which causes embrittlement because of deposition of carbide at the grain boundaries. On the other hand, carbon-free aluminum ferrous alloys are apt to become embrittled by the contamination of alumina inclusions. Therefore, the basic requirement for a high-quality aluminum ferrous alloy is freedom from alumina inclusions as well as less carbon content to such a degree as can be technically attained. Preparing experimental aluminum ferrous alloys, electrolytic iron may be used to meet this requirement, but such iron is too expensive for the production on a commercial scale.

At molten iron temperatures, aluminum is a powerful deoxidizer. This characteristic must be considered when it is used as an alloying element, because an undesirable quantity of alumina inclusions will be present unless precautions are taken. It is due to this fact that special techniques such as vacuum or inert gas melting have conventionally been recommended as the best way to obtain satisfactory results, though they have various disadvantages such as difficulty in operation, necessity of special refractories, etc.

As has already been mentioned, in manufacturing the aluminum ferrous alloys by the method of the present invention, carbon or alloy steel can preferably be used as the starting material in the form of thin elongated members, such as rods having a small diameter, strips or tubes with thin-wall thickness. When the aluminum ferrous alloys are required to contain no special elements other than aluminum, rods of pure metal may likewise be used for their addition. However, all these materials above mentioned not only contain more or less amount of carbon but also there are always present oxides on their surfaces. Precautions must, therefore, be taken to insure that the oxides will completely be reduced, and further that the carbon will be removed as completely as possible.

2

I have found that a heat-treatment of steel in the form of thin elongated members, such as rods, strips or tubes at temperatures above 700° C., in an atmosphere of hydrogen, is a simple and yet effective method of reducing both the carbon content and oxides to a maximum. In the existing methods, molten iron has to be given a decarburizing and deoxidizing treatment with hydrogen, followed by vacuum treatment. Compared with the method of the present invention, the molten methods should be equally effective; but hydrogen is potentially explosive, especially at those elevated temperatures, so that its practical use is limited. By contrast, the solid method is both simple and economical, and yet the carbon content can easily be reduced to a sufficiently low level to obtain ductile aluminum ferrous alloys. Thus, I am, as far as I know, the first to adopt the solid method as a standard procedure prior to alloying iron with aluminum.

To illustrate the method according to the present invention, reference is made to the accompanying drawing in which:

Fig. 1A is a side elevation, partly in section of a batch type furnace with a plurality of steel rods packed therein, the view being taken along line X—X of Fig. 1B;

Fig. 1B is a section along in Y—Y of Fig. 1A;

Fig. 2 is a cross sectional view of an electrode prepared according to the present invention;

Fig. 3A is a sectional view of an apparatus for preparing an electrode according to the method of the present invention;

Fig. 3B is a section through line B—B of Fig. 3A;

Fig. 4 is a sectional view of a modified form of an electrode prepared according to the present invention; and

Fig. 5 is a schematic representation of a consumable electrode electric arc furnace having a water cooled crucible.

To insure the decarburization of those thin, elongated members, a batch type or a tumbling furnace may be used. The batch type furnace consists of a long horizontal heating chamber, in which are arranged a number of tubes made of stainless steel. The arrangement for decarburizing is schematically shown in Fig. 1, which illustrates one of stainless steel tubes to be arranged in the long horizontal heating chamber of a batch type furnace. The steel rods 1 are compactly loaded in lengthwise parallel relationship within the tube 2, through which hydrogen is caused to flow from inlet 3 to outlet 4. In this case, the time needed for complete decarburization depends upon the carbon content, the diameter of rods, temperature and the composition of the atmosphere. As is well-known, moist hydrogen is preferred to dry hydrogen for its decarburizing ability. On the other hand, the tumbling furnace has an advantage which brings a good contact of hydrogen with the rods, resulting in uniform and complete decarburization. It is, however, unsuitable for long rods with excessively small diameter to be treated in such a tumbling furnace, because they are liable to get entangled.

The next step is to prepare a consumable electrode such as are shown in Fig. 2, 3 and 4. To prepare the electrode shown in Fig. 2, the decarburized iron rods 5 are bundled together to make an electrode with a material, the essential constituent of which is aluminum. For example, there may be used substantially pure or alloy aluminum in the form of rods 6 with a small diameter. Then the bundle is forced into a closely fitting iron tube 7 which has equally been decarburized. The tube thus filled up may be usable for a consumable electrode. In this connection, the sealing of the bundle by an iron tube is effective to prevent the ferrous rods from reoxidation, particularly when melting is carried out in the air. Further, it is worth mentioning that a uniform distribu-

tion of aluminum containing rods in the structure of the electrode is the indispensable means to insure a homogeneity of the resulting aluminum ferrous alloys.

Fig. 3 is a view of another type of consumable electrode consisting of iron rods packed in aluminum. To prepare this type electrode, molten aluminum 8 contained in a melting pot 13 of the apparatus of Fig. 3a is sucked into the iron tube 9 by means of a vacuum so as to fill up around the iron rods 10 shown in the cross sectional view of Fig. 3b. The method is effective especially when alloy aluminum is to be alloyed with iron, because high alloy aluminum is too brittle to be drawn to a fine rod.

In both methods above mentioned, the operations are carried out in two parts: steel rods are first heat-treated in an atmosphere of hydrogen, and then combined with aluminum to prepare the electrode. This is due to the fact that, since aluminum melts at 655° C., it cannot be heat-treated together with steel rods at temperatures above 700° C. In this connection, I have found a method of preparing still another type electrode by using effectively steel-clad aluminum rods in place of aluminum rods. The clad rods are made by drawing a steel tube containing an inner core of aluminum. They can be heated at temperatures above 700° C. without becoming brittle or melting, though precautions must be taken lest the temperature should be elevated above 850° C.

As is shown in Fig. 4, the clad rods 14 are bundled together with steel rods 15 and stuffed into a steel tube 16. Then the steel tube is heat-treated in an atmosphere of hydrogen in accordance with the procedure already mentioned. After completing decarburizing, the iron tube containing the clad rods may immediately be used for a consumable electrode. The electrode thus prepared is free from trouble caused by reoxidation of iron rods as well as the difficulty in removal of alumina film existing on the surface of an aluminum. Therefore, the advantages of this type electrode will be noted as follows: 1. Improved chemical homogeneity. 2. Less contamination from alumina inclusions. 3. General simplification and improvement in preparing the consumable electrode.

Lastly, the third step is to melt the consumable electrode by an electric arc in a water-cooled metal crucible. Fig. 5 shows the procedure schematically. As can be seen from this illustration, the consumable electrode 17 is to be melted by electric arc 18 in a water-cooled crucible 19. Though this furnace for casting high aluminum-iron alloys is substantially similar to those which are generally used for titanium or zirconium, in the furnace employed by the present invention neither vacuum nor inert atmosphere is absolutely needed. I have found that, at least so far as the ductility and oxidation resistance are concerned, melting in air is good enough to obtain a satisfactory resulting product. Therefore, the construction of the furnace is very simple, and it is possible to cast a continuous ingot 20 by using a retractable bottom 21.

Further, the invention is illustrated by the following examples in which the compositions of the starting materials used were as follows:

- (1) Steel rod 2 mm. in diameter; 0.25% C, 0.42% Mn, 0.04% P, 0.03% S.
- (2) Steel tube 2 mm. in wall thickness; 0.16% C, 0.35% Mn, 0.03% P, 0.03% S.
- (3) Stainless steel rod 3 mm. in diameter; 18.5% Cr, 0.07% C.
- (4) Aluminum rod 2 mm. in diameter; 99.7% Al.
- (5) Silumin; 15% Si, 85% Al.

#### Example 1

The steel rods and tubes were heated at 750° C. in an atmosphere of moist hydrogen for 15 hours. The treated rods were bundled together with aluminum rods and forced into the tube to prepare a consumable electrode. The resulting alloy containing 10.5% aluminum could be either hot or cold worked without difficulty. The wire

drawn to 1 mm. in diameter had a tensile strength of 62 kg./mm.<sup>2</sup> and the elongation was 35% on measuring on 20 mm. gauge length.

#### Example 2

The steel rods and tubes were heated at 800° C. in an atmosphere of hydrogen for 24 hours. The resulting alloy containing 14% aluminum could be cold rolled to 1 mm. thickness sheet and drawn to 1 mm. diameter wire.

#### Example 3

The stainless steel rods were heated at 800° C. in an atmosphere of moist hydrogen for 20 hours. The resulting alloy contained 10.5% aluminum and 2.5 chromium, and was ductile enough to be cold worked without much difficulty. This ternary alloy has extremely good resistance to oxidation at temperatures as high as 1200° C.; at least as good as the binary alloy containing 15% aluminum.

#### Example 4

The steel rods and tubes were hydrogen-treated at 800° C. for 20 hours. After the decarburization was completed, molten aluminum alloy containing 15% silicon was sucked into the iron tube by means of the vacuum method to fill up around the rods. The resulting alloy contained 13% aluminum and 2% silicon. It could easily be cold rolled to 1 mm. thickness sheet.

#### Example 5

The diameter of clad rods used was 4 mm., that of aluminum cores being 2 mm. 26 pieces of the clad rod were stuffed into a closely fitting tube 32 mm. in inner diameter and 1 mm. in wall thickness. The tube was treated by hydrogen at 750° C. for 15 hours. The resulting alloy contained 7.6% aluminum, and was ductile enough to be cold drawn to 0.2 mm. thickness with ease.

The descriptions are intended to be illustrative only and it is to be understood that changes and variations may be made without departing from the spirit and scope of the invention as defined by the appended claims.

I claim:

1. A method of manufacturing ductile high aluminum ferrous alloys containing up to 18% aluminum, comprising the steps of heating a ferrous alloy while it is in a solid state to a temperature in excess of 700° C. in an atmosphere of hydrogen for decarburizing said ferrous alloy, preparing an electrode by combining the thus decarburized ferrous alloy and a material consisting essentially of aluminum, and using the thus prepared electrode as an electrode in an electrode type arc furnace to cast an ingot in a water cooled metallic crucible.
2. A method of manufacturing ductile high aluminum ferrous alloys containing up to 18% aluminum, comprising the steps of preparing an electrode by combining a ferrous alloy and a material consisting essentially of aluminum, heating the thus prepared electrode while it is in a solid state to a temperature in excess of 700° C. in an atmosphere of hydrogen for decarburizing the ferrous alloy in said electrode, and using the thus decarburized electrode as an electrode in an electrode type arc furnace to cast an ingot in a water cooled metallic crucible.
3. A method of manufacturing ductile high aluminum ferrous alloys containing up to 18% aluminum, comprising the steps of heating a plurality of thin elongated steel members to a temperature of from 700 to 850° C. in an atmosphere of hydrogen, preparing an electrode by forcing the thus decarburized elongated members together with elongated aluminum containing rods into a tube of decarburized ferrous material, and using the thus prepared electrode as an electrode in an electrode type arc furnace to cast an ingot in a water cooled metallic crucible.
4. A method of manufacturing ductile high aluminum ferrous alloys containing up to 18% aluminum, comprising the steps of forming an electrode by inserting a plu-

rality of thin walled steel tubes having an inner core of aluminum and a plurality of slender steel rods into a thin walled steel tube, heating the thus formed electrode to a temperature of from 700 to 850° C. in an atmosphere of hydrogen to decarburize said electrode, and using the thus decarburized electrode as an electrode in an electrode type arc furnace to cast an ingot in a water cooled metallic crucible.

5. A method of manufacturing ductile high aluminum ferrous alloys containing up to 18% aluminum, comprising the step of heating a plurality of thin elongated steel members to a temperature of from 700 to 850° C. in an atmosphere of hydrogen, preparing an electrode by

placing the thus decarburized members in a thin walled tube of decarburized ferrous material, placing molten aluminum containing material in said tube around the thin elongated members therein, and using the thus prepared electrode as an electrode in an electrode type arc furnace to cast an ingot in a water cooled metallic crucible.

## References Cited in the file of this patent

## UNITED STATES PATENTS

|    |           |                |               |
|----|-----------|----------------|---------------|
| 10 | 2,159,169 | Mautsch        | May 23, 1939  |
|    | 2,234,127 | Mautsch        | Mar. 4, 1941  |
|    | 2,319,977 | Cape et al.    | May 25, 1943  |
|    | 2,631,118 | Boothby et al. | Mar. 10, 1953 |